

March 28, 1933.

W. T. ANDERSON, JR.

1,902,936

ELECTRODE FOR VAPOR GAS ELECTRIC DEVICE

Filed March 8, 1932

*Fig. 1*



*Fig. 3.*



*Fig. 2.*



INVENTOR.

William T. Anderson, Jr.  
BY Frank C. Fischer.  
ATTORNEY.

## UNITED STATES PATENT OFFICE

WILLIAM T. ANDERSON, JR., OF NEWARK, NEW JERSEY, ASSIGNOR TO HANOVIA CHEMICAL AND MANUFACTURING COMPANY, OF NEWARK, NEW JERSEY, A CORPORATION OF NEW JERSEY

## ELECTRODE FOR VAPOR GAS ELECTRIC DEVICES

Application filed March 8, 1932. Serial No. 597,481.

This invention relates to electrodes for vapor gas electric devices. These electrodes may be employed on the familiar forms of mercury arcs, both vacuum and gas filled type, for the production of light and for rectification, and they may be used for gas discharge tubes for the production of light.

The invention covered by this application is generally described and shown, but not 10 claimed, in Letters Patent No. 1,890,926 issued Dec. 13, 1932, on an application filed June 16, 1931, by myself and Hugh D. Fraser.

My invention relates in particular to temperature control of electron emitting electrodes and in order that the importance and 15 significance of such control may be thoroughly understood, it is necessary to describe the conditions existing in and at the electrodes of mercury arcs and gas discharge tubes.

20 The electrode of an air-cooled quartz mercury vapor arc, which is a familiar article of commerce, consists of a quartz vessel containing mercury connected to the outside current supply by means of a vacuum sealed lead-in wire. The arc discharge is from the surface of the mercury. The arc possesses a negative volt-ampere characteristic, that is, the current decreases as the voltage increases, and is 25 not to be confused with a high electron discharge which has a positive volt-ampere characteristic resulting in high voltage and low amperage. The typical arc which will be described operates at 300 watts and 4.2 amperes 30 in the arc itself.

35 The electron emission and the mercury vapor which maintain the arc result from the temperature produced at the vapor discharge metallic mercury interface. The initial high 40 temperature that starts the arc is created by short circuiting the mercury electrode to the other electrode which may be mercury or some other substance. The area of the vapor discharge metallic mercury interface is very 45 small, being about 0.0012 square centimeter for the 4 ampere arc. (For a 20 ampere arc it would be about 0.005 square centimeter.)

The temperature at this discharge to mercury contact is about 2270 degrees centigrade, 50 at the best operating conditions. The vapor-

ization of the mercury from the electrode at the contact area is about  $7.20 \times 10^{-8}$  grams per second per ampere, which results in a total mercury pressure at the electrode of the order of  $2\frac{1}{2}$  atmospheres.

55 Not all the heat generated at the "hot spot" is employed for electron emission and mercury vapor production. Some of the heat is employed to warm the entire electrode, and some is radiated or conducted to the walls of the electrode where it is dissipated. Mercury vapor is also condensing in the cooler parts of the container, liberating heat. Finally an equilibrium is established, the final temperature of the system depending upon the current, radiation and thermal conductance.

60 Efficient operation demands that this equilibrium temperature be restricted to within certain rather narrow limits. It is characteristic of the mercury arc that when the temperature is lowered, the amperage of the arc increases, and vice versa, an increase in temperature results in a decrease in amperage. If the temperature be lowered to too great 65 an extent, the high resulting amperage will result in rapid deterioration of the glass or quartz container. On the other hand, if the temperature be increased too much, the amperage may become too low to maintain the 70 "hot spot", and the arc will be extinguished. Between these two points the arc may be operated with various degrees of efficiency.

75 Temperature in commercial arcs is controlled by limitation of arc current, radiation and provision for adequate electrode 80 cooling surfaces. The electrode surface employed with this typical 300 watt air cooled mercury arc has a surface area of about 4375 square millimeters and contains a volume of 85 mercury about 21,980 cubic millimeters, representing in weight about 300 grams of mercury. This surface may be cooled by natural air convection currents, or the air cooling may be assisted by metal cooling vanes.

90 I have found that the size and design of these mercury electrodes is dependent in a large measure on the low thermal conductivity of metallic mercury. Mercury in a layer one centimeter deep and an area one square 95 centimeter transmits only 0.019 calorie per 100

second for an increase in temperature of one degree centigrade. Under similar conditions copper transmits 1.00 calorie per second, aluminum 0.50 calorie per second, tungsten 0.48 calorie per second, molybdenum 0.34 calorie per second. Thus the thermal conductivity of copper is about 50 times higher than that of mercury.

As a result of this low thermal conductivity, the temperature gradient within the mercury electrode is very great, and hence a correspondingly greater volume of mercury and a greater surface area are required than would be necessary if the electrode contained, for instance, copper instead of mercury.

It is an object of the invention to provide mercury electrodes which compensate for the low thermal conductivity of the mercury metal, and which are equal in efficiency or better than those familiar to commerce, but much smaller in size and volume. The decrease in size and volume has resulted in a saving in mercury which in the final highly purified form required for use in such arcs is one of the most costly items employed in the manufacture of these arcs. Also, if the envelope be constructed of transparent fused quartz a reduction in the size effects another economic saving.

Aside from these advantages resulting from my invention, there are others resulting from a reduction in electrode size. When such electrodes are employed on mercury arcs for the production of light they permit a compactness which especially adapts such an arc for use with reflectors. A suitable reflector located behind a mercury arc can greatly enhance the intensity of light falling upon a surface. If the light source is compact and free from appreciable obstructions to light, the reflector design is greatly simplified.

My invention, since it enables the employment of electrodes of half to one-third the size of those employed on older arcs of this type, can be more easily and satisfactorily employed in conjunction with reflectors. Another advantage resulting from the employment of my invention relates to lessened breakage in shipment.

The vacuum type quartz mercury arc in particular may be broken in shipment by a mercury slap which results from the heavy mercury metal being suddenly thrown from one end of the container to the other. The number of such lamps that are broken by this cause is in direct proportion to their size and the volume (and hence the weight) of mercury contained therein. My invention permits a reduction of the amount of mercury in these lamps and will therefore result in smaller sized arc tubes.

In the drawing,  
65 Figure 1 represents a sectional view of an

electrode employing an alkaline earth metal and embodying the invention, and,

Figure 2 represents a sectional view taken on line 2—2 of Figure 1,

Fig. 3 is a perspective view of an electrode 70 mass having metallic heat conducting means distributed therein.

I have studied and operated vapor electric devices containing mercury which produce light radiations in every respect similar to the ordinary familiar mercury arc, and which have the same electrical characteristics as the mercury arc, namely, a negative volt-ampere relationship, the arc current decreasing as the arc voltage increases, but whose operation was dependent primarily upon electron emission by substances other than mercury, and in this respect different from the ordinary mercury arc.

The electrodes in this type of lamp contain the alkaline earth oxides such as barium and strontium oxides as their primary active electron emitting substances.

The employment of these substances for the purpose of electron emission is not new 90 as they were used for such purposes as early as 1914. However, the manner in which I employ these oxides, and the light source which I obtain by their use I believe to be a novel and distinctive advance in the art of 95 light production.

This new type of electron emitting electrode for employment in mercury arcs may be made as follows. The alkaline earth oxides in a finely powdered form are thoroughly mixed with granulated metallic oxides, which as metallic hydroxides in aqueous solution, give an electrolytic dissociation of low hydroxyl ion concentration. Typical oxides are ferric oxide, chromic oxide, aluminum oxide, zirconium oxide, nickel oxide, cobalt oxide, and titanium oxide etc. The proportion of alkaline earth oxide to metallic oxide is dependent upon the design and current duty of the electrode.

This mixture is made into a paste with an organic binder such as cellulose acetate in ether-alcohol solution. The paste is moulded on the lead-in wire which may be tantalum, molybdenum or tungsten. The moulded electrode is dried in a vacuum, and then heated in a silica tube to about 1000 degrees centigrade to carbonize the binder; and to weld the mass together still further, the electrode is glowed for a few seconds in the oxy-hydrogen reducing flame. The finished electrode is introduced into the electrode vessel, and the lead-in wire is sealed gas tight to the vessel.

The weak basic metallic oxides have been 125 found useful in the construction of these electrodes because of their stability at the operating temperatures (approximately 1100 degrees centigrade excepting "hot spot" which is higher temperature) and their 130

ability to adsorb barium and strontium oxide molecules on their surfaces.

This adsorption property may result from their weak basic properties, for in aqueous 5 solution and in a few instances in crystalline hydrated form, investigators have isolated and identified chemical compounds resulting from combination between these oxides and the alkaline earth oxides. However, at incandescence there is no evidence that true 10 chemical union exists between these substances, and their association in these electrodes which operate at incandescence should be considered one of adsorption and physical 15 mixture.

The adsorption of the alkaline oxides on the surfaces of the metallic oxides may be considered analogous to the adsorption of gases on metallic catalysts in gas reactions 20 such as the ammonia synthesis. The adsorption results in a distorted electron field in the alkaline earth molecule, and when an electric potential is applied, electrons may be discharged. The electron emission occurs at 25 relatively low temperatures, that is, at room temperature, when the combinations described are employed. These weak basic metallic oxides are employed then as non-volatile supports and as creators of electron 30 emission centers operative at low temperatures.

The completed electrodes are attached to the body of the lamp proper. Two electrodes are sufficient for either alternating or direct 35 current operation. The assembled lamp is attached to an evacuation and filling system, and is evacuated. While on the vacuum system, the lamp is heated by the external application of heat to drive off moisture and 40 gases adsorbed on the walls. Finally the system is cooled on the vacuum and a small quantity of mercury, more than sufficient to supply all the mercury vapor needed for arc operation, but very little in excess, is admitted.

45 Since there is too little mercury in the system to permit the establishment of the arc by the familiar method of tilting the burner so that mercury can flow from one electrode to the other, short circuiting the system, it is necessary to provide a means for lighting the 50 lamp. This has been accomplished by introducing into the system a small quantity of neon gas at a pressure of a few centimeters. If now the arc tube be gently stroked with 55 a cloth to produce an electrostatic charge on the tube, a few neon ions will be formed.

If the two electrodes are maintained at a 60 potential difference greater than 150 volts, a gas discharge will be formed which will almost instantaneously volatilize sufficient mercury and establish sufficiently high electron emission to permit the mercury arc to establish. The instant that the mercury arc is started, the voltage drops, and the gas discharge ceases to function.

From this point, the gas ceases to play any part in the operation of the arc, the arc appearing in every respect to resemble the ordinary mercury arc.

It is essential that during operation that 70 the arc voltage be maintained below the ionization potential of the gas, as otherwise the electrodes will flash over. The starting voltage and also the flashing voltage are characteristic of the physical dimensions of the lamp, and hence vary somewhat for lamps 75 of different sizes. The lamp referred to has an arc length about 8 inches.

This lamp is operated and the arc is maintained by the emission from a "hot spot" on the electrode. Similarly, if the current supply is interrupted for a very short time, the arc is extinguished, and will not start of its own accord. However, unlike the mercury electrode type, the alkaline earth oxide type 80 cannot be relighted immediately, for there is not sufficient emission to re-establish the arc in the mercury, and the vapor pressures within the neighborhood of the electrodes interfere with the action of the inert gas. The 85 lamp must cool before it can be lighted again. 90

Lamps, such as described, have proven not satisfactory articles of commerce because they deteriorate too rapidly. This deterioration results from the rapid and continuous disintegration of the electrodes. I have found the cause for this rapid destruction of the electrodes to be that the electrodes become too 95 hot.

The alkaline earth oxides, barium and 100 strontium oxides, and also the metallic oxides have thermal conductivities of the order of 0.0123 calorie per second through a layer one centimeter deep and an area one square centimeter for an increase in temperature of one degree centigrade. This means that they are even poorer conductors of heat than mercury. There is the characteristic "hot spot" from 105 which the electrons are emitted. In this instance there is not any mercury at the electrode to evaporate. 110

All the heat energy generated must be dissipated from the electrode itself. The electrode therefore becomes very warm, and volatilization of the alkaline earth oxides becomes a result. Whereas the volatilization of appreciable mercury from the mercury type of electrode is without serious consequences, any appreciable volatilization of the alkaline earth oxides will result in greatly 120 shortened useful life.

At the time the electrode is moulded, a series of layers of metal gauzes, foils, or spirals of metals which have high thermal conductivity are introduced into the mass. 125 These metals may be tungsten or molybdenum.

These layers or spirals are connected and arranged in such a way that when the electrode is seated in the electrode vessel they 130

make contact with the walls. They are thus enabled to conduct the heat from the electrode to the walls which in turn may be cooled by any familiar method, such as metal 5 cooling vanes.

Referring to the drawing, there is shown an electrode mass 2 which is made from a mixture of alkaline earth oxides and metallic oxides, as hereinbefore explained. The alkaline earth oxides may be of barium or strontium; and the typical metallic oxides are ferric oxide, aluminum oxide, nickel oxide, cobalt oxide, etc. The electrode mass 2 has layers of metallic gauze 3 distributed 10 therein, and contacting with the wall of a silica sleeve 1 surrounding the electrode. The sleeve 1 is sealed to the electrode vessel 5, the latter carrying a quantity 6 of mercury between its wall and the wall of the 15 sleeve. A lead-in wire 4 is sealed into the electrode vessel and embedded in the electrode mass 2.

Employing electrodes constructed in accordance with my invention, it is possible 20 to construct mercury arc lamps for the production of visible and ultra violet light and for current rectification which compare in electrical and radiation characteristics comparable to the familiar mercury electrode 25 types of arcs and which have some advantages not enjoyed by the older type of arc. Thus the lamp may be operated directly on alternating current by applying potential to two electrodes only whereas the ordinary 30 mercury arc requires three electrodes for such operation. The very small quantity of mercury in the new lamp enables the lamp to be operated in any position, and also results in ease of shipment.

40 Having thus described my invention, what I claim as new and desire to secure by Letters Patent, is:

1. An electrode for vapor electric devices, comprising a gas tight vessel, an electrode 45 mass formed of alkaline earth oxide intimately mixed with weakly basic metallic oxides, a sleeve surrounding said electrode mass, and a plurality of pieces of metal distributed throughout the electrode mass and 50 contacting the wall of the sleeve, said metal pieces being of higher thermal conductance than the electrode mass to conduct a portion of the heat of the electrode mass to the wall of the sleeve.

55 2. An electrode for vapor electric devices, comprising a gas tight vessel, an electrode mass formed of barium and strontium oxides intimately mixed with particles of the oxides of iron, chromium, aluminum, nickel, cobalt, 60 zirconium, titanium and zinc, a lead-in wire of metallic tungsten sealed into the vessel and embedded in the electrode mass, a sleeve surrounding the electrode mass and sealed to the vessel, and pieces of tungsten metal gauze 65 distributed throughout the electrode mass,

and contacting the sleeve to conduct heat from the electrode mass to the sleeve and thence to the vessel.

3. In an electrode for vapor electric devices, an electrode mass formed of alkaline earth oxides and metallic oxides, a sleeve surrounding said electrode mass, and a plurality of pieces of metal gauze distributed throughout the electrode mass and contacting the sleeve to conduct heat from the electrode 70 mass to the sleeve.

4. An electrode for vapor electric devices, comprising a gas tight vessel, an electrode mass formed of alkaline earth oxides and metallic oxides, a lead-in wire sealed into the vessel and embedded in the electrode mass, a sleeve surrounding the electrode mass and sealed to the vessel, and pieces of metal distributed throughout the electrode mass and contacting the sleeve to conduct heat from 80 the electrode mass to the sleeve.

5. In a vapor electric device having a gas tight vessel containing a small quantity of mercury, and a rare gas for the purpose of establishing the mercury arc, an electrode 90 comprising an electrode mass formed of alkaline earth oxides and metallic oxides, a lead-in wire sealed into the vessel and embedded in the electrode mass, a sleeve surrounding the electrode mass and sealed to the vessel, and pieces of metal distributed throughout the electrode mass and contacting the sleeve to conduct heat from the electrode mass to 95 the sleeve.

This specification signed this 29th day of 100 February, 1932.

WILLIAM T. ANDERSON, JR.

105

110

115

120

125

130